

## UNITED STATES PATENT OFFICE

1,968,067

## ALLOY AND METHOD OF MAKING SAME

Clarence W. Balke, Highland Park, Ill., assignor,  
by mesne assignments, to Ramet Corporation  
of America, North Chicago, Ill., a corporation of  
Illinois

No Drawing. Application May 29, 1930,  
Serial No. 457,496

13 Claims. (Cl. 75—1)

This invention relates in general to alloys and a method of producing the same, and while it has generally for an object the provision and production of an extremely hard and strong alloy 5 having very great wear resisting qualities, the invention has more particular reference to the provision and production of alloys composed of a refractory metal and a metalloid, which will adapt such alloys for use in the formation of tools for 10 cutting and working other metals.

The invention contemplates the provision of a very hard alloy comprising a refractory metal, such as tantalum, columbium or tungsten chemically united with a metalloid, such as boron. 15 This boride is heat treated with another metal to provide an alloy suitable for the formation of metal cutting or working tools, or as wire drawing dies.

Alloys for the formation of metal cutting and 20 working tools have heretofore consisted of various combinations of metals with the refractory metals and carbon. While such alloys possess a high degree of hardness and wear resisting qualities, it has been found that a refractory metal 25 boride combined with an auxiliary metal is considerably harder and possesses the desirable qualities which are requisite in metal working or cutting tools and wire dies.

It is a primary object of this invention to produce 30 a tantalum boride alloy and a method of producing such an alloy.

An important object of the invention is the provision and production of a hard metal alloy which includes boron and a refractory metal.

35 Another important object of the invention is the production of a novel alloy, comprising a refractory metal, the boride of the refractory metal, and another metal.

Other objects and advantages of the invention 40 will be apparent from the following description which discloses a preferred embodiment of the invention.

The novel method for producing the extremely 45 hard alloy of the present invention briefly comprises uniting a refractory metal powder, such as tantalum, columbium, molybdenum, or tungsten powder with boron, which has been preheated to purify it. It will be understood that amorphous boron and various chemical compositions which 50 will give boron when heated, such as the composition having the chemical formula of  $B_6C$ , are here contemplated as coming within the scope of the present invention. The refractory metal 55 powder and the boron are then heated in an evacuated electric furnace and are ground to a very finely divided powder. This finely divided powder is next mixed with a hydrogen reduced metallic powder of one or more metals of the 60 iron group, and the boride and metallic powders

are very thoroughly mixed and ground to an extremely finely divided powder.

After thoroughly mixing the boride powder with that of the metal or metals of the iron group and grinding them to a very finely divided form, the mixture is then subjected to tremendous pressure to form a substantially non-porous and homogeneous body of the desired size and shape. This non-porous and homogeneous body is subjected to a heat treatment in a vacuum at 70 from 1350° to 1400° C.

This heat treatment serves to combine the degasified constituents in the form of a solid homogeneous alloy having an exceedingly fine grain and providing a very hard composition suitable 75 for use in the manufacture of metal cutting or working tools and wire dies, and for other uses requiring an alloy having wear resisting qualities combined with extreme hardness and great strength.

80 Attention is here directed, before proceeding with the disclosure of the invention, to the tremendous pressure referred to above in forming the mixed and ground powders into a homogeneous body having a relatively fine grain. This pressure is sufficient to permit handling and readily forming the body to a desired shape and size prior to the heat treatment, which combines or unites the constituents of the alloy, and in practice, a pressure of about eighty tons per square 85 inch is used.

85 In carrying out the invention to accomplish the above mentioned objects, it is desirable to provide a sufficient quantity of the refractory metal that some of it may combine with the metalloid and the remainder with another metal forming the alloy.

90 The boron employed to produce the boride is preferably in the form of amorphous boron which has been preheated to about 1500° C. to 95 volatilize any organic matter contained in the boron and to rid it of objectionable gases. After such purification, the boron is mixed with a refractory metal powder, such as tantalum powder in about the proportion of from 3 to 6% boron and 97 to 94% tantalum by weight. This mixture is ground and mixed in a ball mill and then placed in a cylinder or crucible of tantalum sheet with a tight fitting tantalum cover.

100 The loaded tantalum cylinder is placed in a graphite crucible and completely surrounded with tantalum powder in order to prevent oxygen or nitrogen from the air from passing into the tantalum boron mixture. The carbon crucible is then placed in graphite and heated in a high frequency furnace by slowly raising the temperature to about 2000° C. and maintaining this temperature for about one-half hour to chemically 105 unite the boron and tantalum. When this crucible of carbon has been heated sufficiently to be- 110

115

120

come red hot, a very violent and explosive reaction takes place, so that possibly a part of the boron powder may be blown out of the reacting mixture.

5 The tantalum boron composition that results from the foregoing uniting operation is a tantalum boride having from 3 to 6% by weight of boron, and after cooling is brownish-grey in color. This powder is exceedingly hard and 10 readily scratches the various hard metal alloys now used for the formation of cutting tools. This tantalum boride is next ground in a ball mill for about twenty-four hours to a finely divided powder and heated to from 1600° to 1700° 15 in a vacuum furnace to degasify and to complete the reaction between the refractory metal and the boron. The boride powder may be subjected to sufficient pressure to hold the particles together under the action of the vacuum pump 20 before subjecting it to the foregoing heat treatment. This latter heat treatment also serves to reduce air spaces among the particles of the powder.

The boride is then ready for mixing with an 25 auxiliary metal to form a homogeneous alloy. While this auxiliary metal may be any suitable base metal having a fusing or sintering temperature below the melting point of the boride, and which will alloy with the refractory metal used 30 at a comparatively low temperature, the present embodiment of the invention contemplates the provision of one or more metals of the iron group, such as, iron, nickel and cobalt. Preferably from 3 to 15% by weight of a hydrogen reduced nickel 35 powder in finely divided form is used in the alloy, although a mixture of nickel powder and iron powder, comprising from 3 to 15% by weight of the composition has been found to produce a very hard alloy which gives excellent results 40 when formed as a tool.

As already mentioned, from 3 to 15% by weight of hydrogen reduced nickel powder is mixed with the boride powder; for example, tantalum boride, and this mixture is ground for 45 about ninety hours in a ball mill to an extremely fine powder, the particles of which are thoroughly and uniformly mixed tantalum boride and nickel.

This mixture is next subjected to a tremendous pressure to the order of about eighty tons per square inch, sufficient to press the powder mixture into a body, which may be handled and formed, or worked to the desired shape and size. When this powder mixture has been so formed, it 50 is heated in a vacuum at from 1350° to 1400° C. and this temperature maintained for about one hour. The resulting alloy has a very fine grain due to the degasifying of the boride, the thorough mixing of the fine powders, the tremendous pressure used to press the mixture for forming prior to the last heat treatment and to the final heat treatment in the vacuum.

One of the alloys made by the foregoing method comprises the following percentages by weight of the materials indicated:

|                                                                       | Percent |
|-----------------------------------------------------------------------|---------|
| Nickel                                                                | 3-15    |
| Tantalum boride                                                       | 97-85   |
| Another alloy contemplated as within the scope 5 of the invention is: |         |
| Nickel, by weight                                                     | 3-15    |
| Tantalum boride, having from 3-6% boron by weight                     | 97-85   |
| 5 Knowledge of the theory of producing a refrac-                      |         |

tory metal boride having an excess of the refractory metal is not necessary to a complete understanding of this invention, and it will be understood that the invention is not limited by the recitation of a possible explanation of this hard and wear-resistant alloy. It is believed that some of the tantalum of the boride is chemically free and combines with the nickel or auxiliary metal to provide an extremely hard bond or cementing material for the tantalum boride, and that this free or uncombined portion of the refractory metal may be considered as being the excess of that required to form the boride of the refractory metal.

Thus, a novel alloy is produced which is sufficiently hard to be used in the formation of metal cutting and working tools, and wire drawing dies. Tools made of this alloy will scratch the tools in use at present, and yet are sufficiently strong and durable or wear resisting as not to crumble, break or chip readily when used as a tool, such as a wire drawing die, to cut or work other hard metals.

Having thus described my invention, what I claim is new and desire to secure by Letters Patent of the United States, is:

1. A hard alloy composed of a tantalum boride, and from 3 to 15% of an auxiliary metal of the iron group.

2. An alloy consisting of tantalum boride and substantially 8% of nickel.

3. An alloy comprising from 3 to 15% nickel and the remainder tantalum and boron in proportion of from 3 to 6% boron and 97 to 94% tantalum.

4. A method of producing a hard alloy of tantalum which comprises heat treating a mixture of tantalum and boron in a vacuum, mixing a powdered auxiliary metal of the iron group with the boride thus formed, and heating the auxiliary metal and the tantalum boride in a vacuum.

5. A method of producing a hard tantalum alloy which comprises chemically uniting tantalum powder with boron, heat treating the tantalum boron composition in a vacuum, pressing a powder of a metal of the iron group with said tantalum boron composition, and heating the mixture in a vacuum.

6. A hard and tough alloy consisting of from 85% to 97% of degasified tantalum boride and from 15% to 3% by weight of nickel.

7. A hard and tough composition composed of tantalum boride alloy including tantalum boride having a boron content ranging between 3% and 6% by weight of said boride, and a metal of the iron group making up from 3% to 15% by weight of the alloy.

8. A hard composition composed of an alloy of a hard refractory metal boride including a boride of a hard refractory metal from the group composed of tantalum and columbium, and an auxiliary metal of the iron group making up from 3% to 15% by weight of the alloy, said boride of said hard refractory metal having a boron content ranging from 3% to 6% by weight of the boride.

9. A hard alloy consisting of a boride of a hard refractory metal from the group composed of tantalum and columbium, said boride making up from 85% to 97% by weight of the alloy, and one or more metals of the iron group making up from 15% to 3% by weight of the alloy.

10. A method of producing a hard alloy of a metal from the group composed of tantalum and columbium, which comprises heat-treating a mix-

ture of said metal and boron in a vacuum, mixing a powdered auxiliary metal of the iron group with the boride thus formed, and heating the auxiliary metal and the boride in a vacuum.

5 11. A method of producing a hard alloy of a metal from the group composed of tantalum and columbium, which comprises heat-treating a powder mixture of boron and said metal from said group composed of tantalum and columbium,

10 whereby a boride thereof is formed, mixing a powder of one or more metals of the iron group with said boride, pressing the mixture, and combining the pressed mixture by heating it in a vacuum.

15 12. A method of producing a hard alloy of one or more metals of the iron group with a boride of a metal from the group composed of tantalum and columbium, said boride having a boron content

of from 3% to 6% by weight of the boride, which comprises heat-treating the said boride in a finely divided state to degasify said boride, mixing therewith said one or more metals of said iron group in a finely divided state, and heating 80 the mixture in a vacuum.

13. A method of producing an alloy of a metal from the group composed of tantalum and columbium, with boron and one or more metals of the iron group, which comprises chemically uniting 85 some of said metal from said group composed of tantalum and columbium with said boron, heat-treating the resulting product in a vacuum whereby to degasify it, pressing a powder of said one or more metals of said iron group together with the degasified product, and heating the pressed mixture in a vacuum.

CLARENCE W. BALKE.

95

100

105

110

115

120

125

130

135

140

145

150